

## UNITED STATES PATENT OFFICE.

EDMUND R. BULLOCK, OF ROCHESTER, NEW YORK, ASSIGNOR TO EASTMAN KODAK COMPANY, OF ROCHESTER, NEW YORK, A CORPORATION OF NEW YORK.

## SELF-TONING PHOTOGRAPHIC EMULSION.

No Drawing.

Application filed January 13, 1922. Serial No. 529,079.

To all whom it may concern:

Be it known that I, EDMUND R. BULLOCK, a subject of the King of Great Britain, residing at Rochester, in the county of Monroe and State of New York, have invented certain new and useful Improvements in Self-Toning Photographic Emulsion, of which the following is a full, clear, and exact specification.

10 This invention relates to photographic emulsions and particularly to those of the type known as "printing-out," that is, upon which light makes a strongly visible impression; and still more particularly to the type 15 known as self-toning, that is, in which the image assumes a desirable colored tone in regular photographic treatment without special toning baths.

It has been customary to make self-toning, printing-out emulsions containing gold compounds. I have discovered that if, instead of gold, a tellurium compound, and particularly a complex tellurium salt, is used, an emulsion having desirable properties may be made.

Following is an example of an emulsion embodying my invention. The figures in each case represent parts by weight.

A: Ammonium chloride, 12; soft gelatin,

30 22; water, 1700.

B: Silver nitrate, 36; water, 40.

C: Trisodium citrate, 8; hard gelatin, 22; water, 340.

D: Silver nitrate, 10; citric acid, 18; water, 40.

E: Tellurium dioxide, 1; sodium hydrogen tartrate, 12; water, 250.

Each of the above mixtures is made separately. Mixture A is then heated until the gelatin is dissolved in the water, whereupon solutions A and B are emulsified together, silver chloride being formed, and the resulting emulsion is allowed to set, squeezed through canvas and washed. Mixture C is then heated until the gelatin is dissolved, and solutions C and D are then emulsified together at as low a temperature as possible

without setting the gelatin. Silver citrate is formed in the emulsion thus formed, which is allowed to set and then slightly washed. To dissolve the tellurium dioxide in E, somewhat protracted heating (conveniently in a large flask with reflux condenser attached) is required.

At this step there is formed a complex tellurium salt, presumably sodium-telluryltartrate and probably analogous in chemical structure to tartar-emetic. This solution can be diluted, if desired, to any extent without precipitation, that is, without undergoing hydrolysis. I preferably use it at the dilution stated. Finally the emulsions A+B and C+D are re-melted and mixed with each other and with solution E and coated on a suitable support, usually paper, in the customary way. It may be noted that the emulsion made by A+B and C+D together is a known printing-out emulsion, containing the sensitive silver salts mentioned and some free citric acid. Many other known formulae for printing-out emulsions might be used and mixed with solution E. As free acid is undesirable in some emulsions of this type, the solution E can be neutralized with sodium carbonate when these are used.

The coated emulsion keeps well. It may be printed upon in the manner usual with printing-out papers. Printing is continued until a depth of image such as is usually required with printing-out emulsions is attained. Combined toning and fixing of the image is effected by direct immersion in a limited volume of hypo solution, (for example, one ounce of 15% solution of crystallized sodium thiosulfate to every 15 square inches of emulsion area) followed by a fresh bath of hypo solution of unlimited volume and washing. The second hypo bath is not strictly essential but is found to be desirable for permanency of the print.

It is to be understood that the above is but an example and that I contemplate as included in my invention all such equiva-

2  
lents as fall within the scope of the appended claims.

Having thus described my invention what I claim as new and desire to secure by Letters Patent is:

1. An emulsion containing a sensitive silver salt and a tellurium compound.
2. An emulsion containing a sensitive silver salt and a complex tellurium salt.
3. An emulsion containing a silver halide and a tellurium compound.
4. A self-toning, printing-out emulsion

containing a silver halide and a complex tellurium salt.

5. A self-toning, printing-out emulsion 15 containing silver chloride and a complex tellurium salt.

6. A self-toning printing-out emulsion containing silver chloride and sodium-telluryl-tartrate.

Signed at Rochester, New York, this 7th day of January 1922.

EDMUND R. BULLOCK.